

## 1

3,227,739

BORIC-ACID-ALKYLOLAMINE REACTION  
PRODUCT

Joseph Versteeg, Roselle, N.J., assignor to Esso Research and Engineering Company, a corporation of Delaware  
No Drawing. Filed Aug. 20, 1963, Ser. No. 303,426  
3 Claims. (Cl. 260—462)

The present invention relates to new additives and to improved lubricating oil compositions containing these additives. In particular, it relates to additives formed by reacting certain amine-type compounds with boric acid.

The additives of the present invention are effective as rust inhibitors and, in addition, minimize copper-lead bearing corrosion. Certain prior art inhibitors, though very effective in preventing rust, cannot be used in some applications because of their adverse copper-lead bearing corrosion characteristics. Included in the prior art compounds, which are excellent antirust additives, are amine-type compounds such as amines, hydroxy amines, amino alcohols, and the like. These amine-type compounds exhibit copper-lead bearing corroding tendencies which preclude their use in many applications.

It is an object of this invention to provide an effective antirust additive which, in addition, does not corrode copper-lead bearings. It is an object of this invention to provide lubricating oil compositions containing these improved additives. In the present invention it has been found that solving the problem of copper-lead bearing corrosion involves more than merely neutralizing a rust inhibitor with some type of acid. It has been found that the neutralization in order to be effective must be accomplished by the use of boric acid. As a preferred embodiment of the present invention, it has been found that certain critical concentrations of the boric acid adduct in a lubricating oil result in an unexpectedly superior lubricating oil composition.

The compounds of the present invention are represented by the following general formula:



where  $n$  is an integer from 2 to 3 and R is a  $\text{C}_6$  to  $\text{C}_{24}$  alkyl group.

In preparing the amine-type compounds suitable for use in the present invention, about equal molar proportions of diethanolamine or dipropanolamine and a long-chain, 1,2-epoxide are reacted, under a nitrogen atmosphere, at a temperature in the range of 25° C. to 250° C. for a period of about 15 minutes to 10 hours. Preferably, a temperature of 110° C. and a reaction time of about 2 hours are used. Unreacted starting materials are removed by vacuum distillation.

The 1,2-epoxides will contain from about 8 to 26 carbon atoms. These epoxides are described in FMC Corporation Technical Bulletins, Nos. 72, 73 and 74.

The compounds of the present invention are prepared by reacting the above-described amine-type compound with boric acid. A temperature in the range of about 200° F. to 400° F., preferably 300° F., is used. In general, equal molar proportions of reactants are used.

The present invention will be further understood by the following examples.

## EXAMPLE 1

$\text{N,N}$ -diethanol 2-hydroxy  $\text{C}_{16}$ - $\text{C}_{18}$  amine, which is an antirust additive, was prepared as follows:

Commercially available  $\text{C}_{16}$ - $\text{C}_{18}$  epoxide (made from animal-derived olefin and hydrogen peroxide) was used.

## 2

105 gm. of diethanolamine were placed in a one-liter flask equipped with stirrer, condenser, thermometer and dropping funnel. The amine was heated to 110° C. and then 273 gm. of the epoxide added dropwise over one hour. Stirring was continued for 2 hours at 110° C. and the product, Additive A, cooled (solid at room temperature).

An additive of the present invention was prepared by reacting an oil solution of Additive A with boric acid.

## EXAMPLE 2

100 gm. of the product of Example 1 were placed in a 400 ml. beaker together with 16.2 gm. of boric acid. Heating and stirring were performed until a temperature of 300° F. was reached. The product, Additive B, lost 13.7 gm. weight in the form of vapor (vigorous evolution) and as a result of normal losses on stirrer and thermometer (estimated at 1 to 2 gm.).

Additive B, prepared above, was added to a lubricating oil and tested for its copper-lead bearing corrosion properties. In this test, Additives A and B were compared with lubricating oils containing  $\text{N,N}$ -diethanol 2-hydroxy  $\text{C}_{16}$ - $\text{C}_{18}$  amine neutralized with other acids. This test consists of operating, under control conditions, engines containing different crankcase oils and determining the resulting loss in weight of connecting rod bearings.

The results of this test are shown below:

30

Table I

|                                             | Concentration, Wt. percent | Cu-Pb Bearing Weight Loss, Mg |
|---------------------------------------------|----------------------------|-------------------------------|
| Base Oil 1                                  |                            | 59                            |
| Additive A                                  | 0.5                        | 159                           |
| Additive A Neutralized with 1/1 Mole Ratio: |                            |                               |
| Boric Acid (Additive B)                     | 0.52                       | 71                            |
| Dimer Acid 2                                | 0.74                       | 139                           |
| 40      Mercaptobenzothiazole               | 1.24                       | 1,985                         |

1 Base oil was a fully formulated SAE 10W-30 motor oil.

2  $\text{C}_{35}$  dimer acid commercially available from Emery Industries Inc. as "Empol" 1022.

45 The above results show that the advantage of the boric acid adduct of the present invention is not simply a matter of neutralization but is specific to boric acid.

In order to determine the antirust properties of the present invention, the following test was performed.

## RUST TEST

50 The test is a very severe test designed to predict rusting of hydraulic valve lifters. In this test new 1958 Oldsmobile valve lifters (cast iron containing a small amount of nickel) are disassembled into body and plunger. These pieces are degreased with solvent and are then allowed to dry, 10 grams of test oil are diluted to 100 grams with hexane. Clean and dry test pieces are soaked in a test solution for one hour, removed and air dried for 30 minutes. This leaves a very thin test oil film on the test pieces. An agar gel collar is cast over the bottom half of each of the two lifter pieces. This collar promotes corrosion by masking half of each lifter piece from oxygen available during the test, i.e. it sets up an oxygen concentration cell. The coated pieces are then covered with water which is aerated and held at 110° F. for 20 hours. Both the water and the agar gel contain  $\text{BaCl}_2 \cdot 2\text{H}_2\text{O}$  for added severity. The pieces show rust in two areas. Red rust appears above the agar (exposed to oxygen-rich water) and black rust under the agar (exposed to oxygen-poor water). The two areas are rated for per cent area covered with rust and the ratings for

